

Feb. 7, 1961

D. W. RYKER

2,970,899

AMMUNITION PROPELLANT

Filed Sept. 28, 1955

3 Sheets-Sheet 1

CARBOHYDRAZIDE-  
NITRIC ACID-WATER  
SYSTEM

FIGURE 1



SEMICARBAZIDE-  
NITRIC ACID-WATER  
SYSTEM

FIGURE 2



FIRING RESULTS

CC CHARGES

○ NO FIRE

× FIRE

□ SOLID

BY

INVENTOR.  
DON W. RYKER  
ATTORNEY  
*Stephen M. Stein*

Feb. 7, 1961

D. W. RYKER

2,970,899

AMMUNITION PROPELLANT

Filed Sept. 28, 1955

3 Sheets-Sheet 2

EFFECT OF CHARGE VOLUME ON CHAMBER PRESSURE



FIGURE 3

INVENTOR.  
DON W. RYKER  
BY  
*Stefan M. Stein*  
ATTORNEY

Feb. 7, 1961

D. W. RYKER

2,970,899

AMMUNITION PROPELLANT

Filed Sept. 28, 1955

3 Sheets-Sheet 3

EFFECT OF CHARGE VOLUME ON VELOCITY



FIGURE 4

INVENTOR.  
DON W. RYKER

BY

*Stefan M. Stein*  
ATTORNEY

1

2,970,899

## AMMUNITION PROPELLANT

Don W. Ryker, Woodbridge, Conn., assignor to Olin Mathieson Chemical Corporation, New Haven, Conn., a corporation of Virginia

Filed Sept. 28, 1955, Ser. No. 537,151

6 Claims. (Cl. 52—1)

This invention relates to a propellant and more particularly to a liquid propellant.

The recent trend in propellants for use in the ammunition field has been directed toward those of the liquid type. Liquid propellants are favored because they are easy to store, do not require grain formation, are easily loaded and dispensed and can be used in such manner to utilize substantially all of their potential. There are many known liquid propellants. However all of these are not useful for use in ammunition because they are either unstable, sensitive, brisant, too slow or too fast burning or of an undesirable low or high potential.

An object of this invention is to provide a novel class of liquid propellants. Another object of this invention is to provide a method for making this novel class of liquid propellants. A further object of this invention is to provide compositions utilizing this novel class of liquid propellants useful for ammunition. And a further object of this invention is to provide liquid propellant compositions that are stable, insensitive and slow burning. Other objects will become apparent to those skilled in the art upon reading the following detailed disclosure and description, with accompanying drawings in which

Figure 1 is a graph illustrating the desirable range of mixtures of carbohydrazide-nitric acid-water particularly useful as propellants.

Figure 2 is a graph showing the desirable range of mixtures of semicarbazide-nitric acid-water particularly useful as propellants.

Figure 3 is a graph showing the effect of charge volume of the carbohydrazide nitrate of Figure 1 on chamber pressure, and

Figure 4 is a graph showing the effect of charge volume of the carbohydrazide nitrate of Figure 1 on velocity.

Broadly, the objects of this invention are accomplished by the use of carbohydrazide and/or semicarbazide-nitric acid-water mixtures with or without additives, such as urea, urea mono-nitrate, guanidine nitrate, methanol and benzene.

In one of its aspects the invention may be accomplished by providing a liquid propellant composition consisting essentially of a 100 part composition of about 34 to 64 parts by weight of a substance selected from the group consisting of semicarbazide and carbohydrazide, about 25 to 55 parts by weight nitric acid and about 7.5 to 16 parts by weight water.

A more thorough discussion of the method of making and using the propellants of this invention can be shown by reference to specific examples, illustrating preferred techniques.

## EXAMPLE I.—SYNTHESIS OF CARBOHYDRAZIDE

Carbohydrazide is synthesized by the action of hydrazine on organic carbonates (see C. C. Clark, "Hydrazine," first edition, 1953, page 75, published by Mathieson Chemical Corporation, Baltimore, Maryland) according to the following equation:



For every mole of diethyl carbonate used, two moles plus some excess of hydrazine in the form of an 85% hydrazine hydrate solution is used. The mixture is heated and distilled until the temperature reaches about 120° C. The reaction is then allowed to cool to enable the carbo-

2

hydrazide to crystallize. The crystals are filtered and dried. A yield of about 65-85% is obtained.

## EXAMPLE II.—CARBOHYDRAZIDE-NITRIC ACID-WATER SYSTEM

The required quantities of carbohydrazide and concentrated nitric acid (70%) were mixed to form the desired ratio by slowly adding the nitric acid to the carbohydrazide. Heat and some slight vaporization of the water of the nitric acid occurred. The nitrate salts formed were clear, faintly yellow, viscous liquids.

A liquid reaction product made by use of equimolar quantities of the carbohydrazide and nitric acid was dehydrated by an extraction with ethyl alcohol and then dried over anhydrous magnesium perchlorate in a vacuum dessicator at 10 mm. pressure.

An analysis of the resultant "dried" solution of the mononitrate was performed using the Karl Fisher method and the xylene distillation method for water determination. The ethyl alcohol content was determined by distillation of the liquid salt product with water, oxidizing with dichromate and back titrating the dichromate with ferric sulfate. The purity of the salt was checked with a nitrate determination. The percentages of each ingredient were determined to be (by weight):

|                            | Percent |
|----------------------------|---------|
| Carbohydrazide mononitrate | 87.1    |
| Water                      | 10.8    |
| Ethyl alcohol              | 0.9     |

The properties of the mono and dinitrate of carbohydrazide in the liquid salt form are tabulated as follows:

|                    | Carbohydrazide<br>Mononitrate             | Carbohydrazide<br>Dinitrate                     |
|--------------------|-------------------------------------------|-------------------------------------------------|
| Impact Sensitivity | Insensitive to hammer blow.               | Insensitive to hammer blow.                     |
| Detonability       | Not detonated by small lead azide charge. | Partially detonated by small lead azide charge. |
| Flame Sensitivity  | Ignited by high temperature flame.        | Ignited by high temperature flame.              |
| 40 Solubility in:  |                                           |                                                 |
| Water              | Miscible                                  | Miscible.                                       |
| Ethyl alcohol      | Immiscible                                | Immiscible.                                     |
| Methyl alcohol     | Immiscible                                | Immiscible.                                     |
| Acetone            | Reacts                                    | Reacts.                                         |
| Benzene            | Immiscible                                | Immiscible.                                     |
| 98% Hydrazine      | Heat evolution.                           | Heat evolution, bubbling.                       |

## EXAMPLE III.—SYNTHESIS OF SEMICARBAZIDE

Semicarbazide may be synthesized by various techniques as disclosed in C. C. Clark, "Hydrazine," first edition, 1953, pages 59-61, published by the Mathieson Chemical Corporation, Baltimore, Maryland. The method here used involves the refluxing of urea and hydrazine hydrate in amyl alcohol according to the following equation:



Equal molar quantities of urea and hydrazine in the form of an 85% hydrazine hydrate solution are refluxed at 118° C. for several hours. Water is removed under vacuum until the mixture attains a temperature of 100° C. The molten semicarbazide is then dissolved in methanol, filtered hot and the filtrate cooled with stirring to precipitate the semicarbazide. The semicarbazide is filtered, washed with methanol and dried under vacuum. A yield of 70% semicarbazide melting at 92-95° C. is obtained.

## EXAMPLE IV.—SEMICARBAZIDE-NITRIC ACID-WATER SYSTEM

The required quantities of semicarbazide and concentrated nitric acid (70%) were mixed to form the desired ratio by slowly adding the nitric acid to the semicarbazide. Heat and slight vaporization of the water of the nitric acid occurred. The nitrate salts formed were clear, faintly green, viscous liquids.

An aqueous salt mixture made by use of equimolar quantities of the semicarbazide and nitric acid was concentrated by an extraction with ethyl alcohol. A similar analysis as performed on the carbohydrazide nitrate mixture of Example II was performed on the semicarbazide nitrate mixture and gave the following result (by weight):

|                           | Percent |
|---------------------------|---------|
| Semicarbazide mononitrate | 92.0    |
| Water                     | 7.5     |
| Ethyl alcohol             | 0.7     |

These systems were subjected to ballistic tests in their aqueous solution form with or without additives.

4  
Table II.—Ballistic tests

SEMICARBAZIDE-NITRIC ACID-WATER SYSTEM

| 5                          | System (by weight) |                |       | Charge<br>(cc.) | Velocity,<br>ft./sec. | Pressure,<br>lbs./sq. in. |
|----------------------------|--------------------|----------------|-------|-----------------|-----------------------|---------------------------|
|                            | Semicarbazide      | Nitric<br>Acid | Water |                 |                       |                           |
| IMR <sup>1</sup> (control) |                    |                |       | 50 gr.          | 2,600                 | 49,000                    |
| 57.9                       | 34.0               | 7.5            | 2     | 1,827           | 56,800                |                           |
| 49.2                       | 41.2               | 9.0            | 2     | 1,823           | 54,300                |                           |
| 40.0                       | 48.8               | 10.6           | 2     | 2,014           | 64,800                |                           |
| 32.6                       | 54.8               | 12.0           | 2     | 1,883           | 62,800                |                           |

<sup>1</sup> Nitrocellulose 88.3%, dinitrotoluene 8.8%, K<sub>2</sub>SO<sub>4</sub> 0.6%, diphenylamine 0.6%.

Table III.—Ballistic tests

CARBOHYDRAZIDE AND SEMICARBAZIDE-NITRIC ACID-WATER SYSTEM

| 6                          | System (by weight) |               |                |       | Charge<br>(cc.) | Velocity,<br>ft./sec. | Pressure,<br>lbs./sq. in. |
|----------------------------|--------------------|---------------|----------------|-------|-----------------|-----------------------|---------------------------|
|                            | Carbohydrazide     | Semicarbazide | Nitric<br>Acid | Water |                 |                       |                           |
| IMR <sup>1</sup> (control) |                    |               |                |       | 50 gr.          | 2,600                 | 49,000                    |
| 51.6                       | 1.3                | 35.5          | 10.6           | 2     | 1,751           | 48,900                |                           |
| 50.6                       | 4.6                | 33.7          | 10.3           | 2     | 1,770           | 50,200                |                           |
| 50.2                       | 2.7                | 35.0          | 10.5           | 2     | 1,802           | 55,200                |                           |
| 49.4                       | 3.4                | 36.7          | 10.6           | 2     | 1,843           | 54,500                |                           |
| 49.4                       | 6.7                | 33.0          | 10.1           | 2     | 1,792           | 52,900                |                           |
| 48.2                       | 9.1                | 32.1          | 9.8            | 2     | 1,784           | 52,400                |                           |
| 48.0                       | 4.6                | 35.9          | 10.5           | 2     | 1,919           | 59,900                |                           |
| 1.4                        | 48.7               | 41.7          | 7.5            | 2     | 1,330           | 55,100                |                           |
| 2.4                        | 47.8               | 41.5          | 7.7            | 2     | 1,871           | 52,200                |                           |
| 3.8                        | 46.5               | 41.3          | 7.7            | 2     | 1,826           | 53,100                |                           |
| 5.5                        | 44.0               | 41.1          | 7.9            | 2     | 1,852           | 51,000                |                           |

<sup>1</sup> Nitrocellulose 88.3%, dinitrotoluene 8.8%, K<sub>2</sub>SO<sub>4</sub> 0.6%, diphenylamine 0.6%.

Ballistic tests

Test firings using a carbohydrazide or semicarbazide-nitric acid-water system made by the technique of Examples II and IV were made using a commercially available brass cartridge case (Super X 30-06 caliber) with a centerfire primer (Type 257W) (both manufactured by the Western Cartridge or Winchester Repeating Arms Plants of the Olin Mathieson Chemical Corporation of New Haven, Connecticut). Before loading, the flash hole leading from the primer into the main cavity of the cartridge was covered with a polyethylene disc prior to seating the primer.

Tabulations of the ballistic tests performed for each system are given in Tables I, II and III.

Table I.—Ballistic tests

CARBOHYDRAZIDE-NITRIC ACID-WATER SYSTEM

| System (by weight)         |                |       | Charge<br>(cc.) | Velocity,<br>ft./sec. | Pressure,<br>lbs./sq. in. |
|----------------------------|----------------|-------|-----------------|-----------------------|---------------------------|
| Carbohydrazide             | Nitric<br>Acid | Water |                 |                       |                           |
| IMR <sup>1</sup> (control) |                |       | 50 gr.          | 2,600                 | 49,000                    |
| 51.5                       | 36.8           | 10.8  | 2               | 1,714                 | 46,200                    |
| 50.1                       | 35.9           | 13.0  | 2               | 1,762                 | 55,200                    |
| 49.6                       | 35.5           | 14.0  | 2               | 1,591                 | 41,500                    |
| 56.0                       | 33.6           | 9.5   | 2               | 1,734                 | 46,700                    |
| 59.0                       | 31.8           | 8.4   | 2               | 1,065                 | 45,000                    |
| 61.7                       | 29.6           | 7.9   | 2               | 1,639                 | 44,600                    |
| 48.2                       | 39.5           | 10.5  | 2               | 1,811                 | 56,200                    |
| 43.8                       | 43.8           | 11.6  | 2               | 1,855                 | 59,800                    |
| 38.9                       | 47.6           | 12.6  | 2               | 1,906                 | 60,600                    |
| 35.6                       | 50.3           | 13.4  | 2               | 1,929                 | 58,300                    |
| 34.7                       | 49.0           | 15.6  | 2               | 1,941                 | 65,300                    |
| 34.0                       | 48.1           | 17.2  | 2               | 1,735                 | 43,000                    |

<sup>1</sup> Nitrocellulose 88.3%, dinitrotoluene 8.8%, K<sub>2</sub>SO<sub>4</sub> 0.6%, diphenylamine 0.6%.

35 The systems carbohydrazide-nitric acid-water and semicarbazide-nitric acid-water were further studied to determine the range of concentrations which gave no misfires under the conditions used. The liquids to be fired were prepared by adjusting ethyl alcohol-washed CMN or SMN with the desired amount of water. The amount of alcohol retained by the washed nitrate was less than 1%. Pressures and velocities were not measured during these firings. Results for 1 cc. charges are plotted on Figures 1 and 2. The area bounded by the black lines on each figure indicates the operable 40 positions.

45 In another series of tests under the same conditions the charge volume was varied from 0.5 cc. to 4 cc. of CMN and the pressure and velocity measured. Results are shown on Figures 3 and 4.

50 In attempting to dehydrate the carbohydrazide mononitrate by heating (165° C.), it was found that water was driven off. At the cessation of this water evolution, heating was discontinued. The distillate was opaque milky white and very viscous. Upon standing, it separated into two phases into a clear, colorless, viscous liquid and the white solid. It was found that the solid constituted about 18% of the total weight of the distillate. Repeated attempts at analyzing and classifying this substance were unsuccessful. It was assumed that 55 the solid material was either a decomposition product or a product of molecular rearrangement or both.

60 The white solid behaved as a propellant. This was demonstrated by firing caliber .30 rounds with a charge containing the solid. Table IV shows the results.

Table IV.—Test of CMN dehydration product

| 70                                                     | Propellant Composition |                   | Charge<br>(cc.) | Velocity,<br>ft./sec. | Pressure,<br>lbs./sq. in. |
|--------------------------------------------------------|------------------------|-------------------|-----------------|-----------------------|---------------------------|
|                                                        | Propellant             | Water,<br>percent |                 |                       |                           |
| Carbohydrazide mononitrate (CMN)                       | 10.8                   | 1                 | 1,404           | 43,100                |                           |
| Carbohydrazide mononitrate CMN Dehydration Product 1-1 | 1                      | 1,532             | 47,600          |                       |                           |

The CMN dehydration product was found to be insensitive to the impact of a 2 kilogram weight dropped 80 centimeters. It could not be detonated with a #6 electric blasting cap.

The ballistic results shown above were varied to a more desirable range by adding certain additives to the carbohydrazide and/or semicarbazide-nitric acid-water systems. The addition was carried out by adding the additive to the propellant system, mixing it and then loading cartridge cases with the proper amount of the mixture. A tabulation of the firing tests is seen in Table V.

Table V.—Ballistic tests

## ADDITIVES TO CARBOHYDRAZIDE AND/OR SEMICARBAZIDE-NITRIC ACID-WATER SYSTEM

| System (by weight)         |               |             |       | Additives         | Charge (cc.) | Velocity, ft./sec. | Pressure, lbs./sq. in. |
|----------------------------|---------------|-------------|-------|-------------------|--------------|--------------------|------------------------|
| Carbohydrazide             | Semicarbazide | Nitric Acid | Water |                   |              |                    |                        |
| IMR <sup>1</sup> (control) |               |             |       |                   | 50 gr.       | 2,600              | 49,000                 |
| 51.5                       |               | 34.5        | 10.5  | Urea              | 2.6          | 1,729              | 54,000                 |
| 51.6                       |               | 34.5        | 10.5  | Urea mononitrate  | 2.5          | 1,821              | 56,700                 |
| 50.4                       |               | 33.6        | 10.3  | do                | 4.8          | 1,785              | 52,700                 |
| 49.2                       |               | 32.8        | 10.0  | do                | 7.2          | 1,792              | 47,400                 |
| 48.0                       |               | 32.0        | 9.9   | do                | 9.3          | 1,850              | 58,100                 |
| 51.5                       |               | 34.5        | 10.5  | Guanidine Nitrate | 2.7          | 1,805              | 56,300                 |
|                            | 48.7          | 40.8        | 7.2   | do                | 2.7          | 1,849              | 53,600                 |
| 53.5                       |               | 35.7        | 10.8  | Benzene washed    | 2            | 1,767              | 51,600                 |
|                            |               | 50.5        | 7.5   | do                | 2            | 1,756              | 49,400                 |

<sup>1</sup> Nitrocellulose 88.3%, dinitrotoluene 8.8%, K<sub>2</sub>SO<sub>4</sub> 0.6%, diphenylamine 0.6%.

As seen in the data above the propellant compositions of this invention are aqueous solutions of carbohydrazide or semicarbazide mono or dinitrate or dehydration products or their mixtures with or without additives in trace to substantial quantities of the mixture. The additives may be semicarbazide, carbohydrazide, urea, urea mononitrate, guanidine nitrate, methanol and benzene. By "trace to substantial" quantities is meant anything within in the range of 0.1% to 10% by weight. A "trace" quantity generally results from washing of the aqueous mixture with an additive.

While a detailed description of this invention has been provided, it is realized that those skilled in the art may make modifications in and adaptations of the propellant composition and its method of manufacture described herein without departing from the spirit and scope of this invention. It is, therefore, to be specifically understood that such obvious modifications are to be considered within the scope of the herein described propellant and method of manufacture.

The invention having thus been described what is to be secured by Letters Patent is as follows:

1. A liquid propellant composition consisting essentially of a 100 part composition of about 34 to 64 parts by weight of a substance selected from the group consisting of semicarbazide and carbohydrazide, about 25 to 55 parts by weight nitric acid and about 7.5 to 16 parts by weight water.

2. A liquid propellant composition consisting essentially of a carbohydrazide-nitric-acid-water mixture as indicated by I of Figure 1 of the drawing.

3. A liquid propellant composition consisting essentially of a semicarbazide-nitric-acid-water mixture as indicated by II of Figure 2 of the drawing.

4. The method of developing a projectile propelling pressure within an enclosed chamber which comprises inserting within said chamber a quantity of a composition made up of 100 parts, said composition consisting essentially of about 34 to 64 parts by weight of carbohydrazide about 25 to 55 parts by weight of nitric acid and 7.5 to 16 parts by weight of water, and locally igniting said mixture.

5. A method of developing a projectile propelling pres-

sure within an enclosed chamber which comprises inserting within said chamber a composition made up of 100 parts, said composition containing as its essential ingredients about 34 to 64 parts by weight of a compound selected from the group consisting of semicarbazide and carbohydrazide, about 25 to 55 parts by weight of nitric acid and about 7.5 to 16 parts by weight of water and locally igniting said mixture.

6. A method of developing a projectile propelling pressure within an enclosed chamber which comprises inserting within said chamber a composition made up of 100 parts, said composition consisting essentially of 34 to 64 parts by weight of semicarbazide, about 25 to 55 parts by weight of nitric acid and about 7.5 to 16 parts by weight of water and locally igniting said mixture to cause a burning of the liquid composition therein.

## References Cited in the file of this patent

## UNITED STATES PATENTS

2,455,205 Whetstone et al. Nov. 30, 1948  
2,682,461 Hutchison June 29, 1954

## OTHER REFERENCES

Thiele et al.: Annalen der Chemie, vol. 283, pp. 22, 23. (Copy in Scientific Library.)  
Andrieth: The Chemistry of Hydrazine, John Wiley & Sons, Inc., New York, N.Y. (1951), pp. 168, 175. (Copy in Sci. Lib.)